



US005160507A

**United States Patent** [19]

Horodysky

[11] **Patent Number:** **5,160,507**[45] **Date of Patent:** \* Nov. 3, 1992

[54] **MULTIFUNCTIONAL ESTER-TYPE ADDITIVES FOR LIQUID HYDROCARBYL OR HYDROCARBYLOXY FUEL**

[75] **Inventor:** Andrew G. Horodysky, Cherry Hill, N.J.

[73] **Assignee:** Mobil Oil Corp., Fairfax, Va.

[\*] **Notice:** The portion of the term of this patent subsequent to Apr. 24, 2007 has been disclaimed.

[21] **Appl. No.:** 532,727

[22] **Filed:** Jun. 4, 1990

[51] **Int. Cl.5** ..... C10L 1/18; C10L 1/22

[52] **U.S. Cl.** ..... 44/390; 44/388; 44/386

[58] **Field of Search** ..... 252/47.5, 48.2; 560/147; 44/388, 390

[56]

**References Cited****U.S. PATENT DOCUMENTS**

3,632,510 1/1972 LeSuer ..... 252/35  
3,632,511 1/1972 Liao et al. ..... 252/51.5  
3,697,428 10/1972 Meinhardt et al. ..... 252/56  
3,725,441 4/1973 Murphy ..... 252/33  
4,919,831 4/1990 Horodysky ..... 252/47.5

*Primary Examiner*—Prince Willis, Jr.

*Assistant Examiner*—John F. McNally

*Attorney, Agent, or Firm*—Alexander J. McKillop; Charles J. Speciale; Howard M. Flournoy

[57]

**ABSTRACT**

Ester-type ashless dispersants containing additional integral sulfur-ester moieties which have been found to possess enhanced thermal and oxidative stability are claimed.

**16 Claims, No Drawings**

MULTIFUNCTIONAL ESTER-TYPE ADDITIVES  
FOR LIQUID HYDROCARBYL OR  
HYDROCARBYLOXY FUEL

RELATED APPLICATIONS

This application is related to Ser. No. 253,306, filed Sep. 30, 1988, and is now U.S. Pat. No. 4,919,831.

BACKGROUND OF THE INVENTION

This application is directed to lubricant and fuel additives and compositions thereof. More particularly, this application is directed to liquid hydrocarbyl or hydrocarbyloxy fuels containing an effective multifunctional amount of an ester-type polymer containing additional sulfur ester moieties, thereby providing exceptional dispersant/detergent activity and thermal stability.

The use of ester-containing or polymeric ester or polymeric ester/amide type carboxylic dispersants are well known, such as those described in U.S. Pat. Nos. 3,341,547, 3,632,510, 3,632,511, 3,697,428, or 3,725,441. These have been used in a variety of commercial lubricant and fuel applications for several decades.

The use of sulfur-ester containing additives have been reported in the literature, primarily in polymer stabilizing applications.

However no prior art known to applicant discloses and/or claims lubricant liquid hydrocarbyl or hydrocarby or hydrocarbyloxy fuel compositions comprising ester-type alkenyl succinic anhydride-derived ashless dispersants having additional integral sulfur-ester moieties.

SUMMARY OF THE INVENTION

It has been found that lubricant and liquid hydrocarbyl fuel compositions containing small additive concentrations of ester-type polyalkenyl succinic anhydride-derived ashless dispersants concentrations of ester-type polyalkenyl succinic anhydride-derived ashless dispersants containing additional integral sulfur-ester moieties possess significantly improved thermal and oxidative stability properties when compared to their non-sulfur-ester containing analogs. The sulfur-ester moieties can be introduced in many ways such as (A) during manufacture of the polymeric or oligomeric dispersant by co-reaction of (1) hydrocarbyl dibasic acid or anhydride, (2) polyol such as pentaerythritol, and (3) relatively small amounts of sulfur-containing acid such as 3,3'-thiodipropionic acid or more conveniently by, (B) reaction of (1) preformed polymeric ester dispersant with (2) relatively small amounts of sulfur-containing acid such as 3,3'-thiodipropionic acid. These preformed (intermediate product) ashless dispersants include any polymeric or oligomeric acid, anhydride or acid generating species reacted with a polyol or polyol amine to yield polymeric ester, amide, imide, containing at least one free OH group available for reaction with sulfur containing acid or acid generating species.

It has now been found that the use of these novel ester-type polymers containing additional sulfur-ester moieties provide exceptional multifunctional dispersant/detergent activity, with additional thermal and oxidative stability properties without any deleterious increase in corrosivity or instability commonly expected with sulfur-containing additives.

Each of the major functionalities are believed to exert significant internal synergistic beneficial properties upon the final additive composition. The ester groups are believed to provide the basis for the dispersancy properties and the integral sulfur-ester groups incorporated with the dispersant molecule are believed to provide the additional unexpected thermal and oxidative stability improvements. These benefits are believed to be enhanced as a result of this novel internal synergism.

10 This multifunctional/multipurpose additive approach is believed to have much wider applicability and may include a range of similar structures containing both (a) polymeric, oligomeric (preferably hexenyl, octenyl or decenyl) or hydrocarbyl ester, amide, imide, or mixed ester/amide/imide dispersant groups and (b) sulfur-ester, sulfonyl, or more generally sulfur-carboxyl containing moieties.

15

Accordingly this application is particularly directed to compositions comprising an oil of lubricating viscosity or grease thereof or liquid hydrocarbyl fuel and minor multifunctional amounts (dispersant/detergent-/antioxidant) of a polymeric, oligomeric or hydrocarbyl ester, amide, imide or mixtures thereof containing at least one free OH group and a sulfur-containing acid or acid generating species.

The remarkable benefits of this invention are also expected for a variety of synthetic and mineral oil based lubricants and greases and for hydrocarbon alcoholic, or hydrocarbon and alcoholic fuels intended for use in internal combustion engines or for heating applications. Both the compositions of matter described and the lubricant and fuel compositions containing same are believed to be novel. To the best of our knowledge, these compositions have not been previously used in lubricating oil, grease, or fuel applications.

Of particular significance in the present invention is the ability of the compositions of matter to provide not only resistance to oxidation but also provide improved anticorrosion characteristics.

DETAILED DESCRIPTION OF SPECIFIC EMBODIMENTS

A polymeric ester was reacted with thiodipropionic acid in the presence of hydrocarbon solvent at elevated temperatures until water evolution ceased to be observed in a Dean-Stark trap. The precise nature of the product is not known. The solvent was then removed by stripping under reduced pressure.

Useful polymeric esters also include those made from dimer acids such as dimerized linoleic acid, dimerized oleic acid and the like, polypropyl succinic anhydrides or acids or other similar acid or acid-generating compositions. Useful polymeric esters also include those made using other polyols or polyhydric alcohols such as trimethylolpropane or dipentaerythritol or tripentaerythritol or mixtures thereof as the polyol source, or tris(hydroxymethyl)aminomethane. Typically the polyhydric alcohols include those containing 6 to about 30 carbon atoms and from about 3 to 6 hydroxyl groups.

Useful sulfur-ester generating species include 3,3'-thiodipropionic acid, dithiodipropionic acid, thiobutananoic acid, similar sulfur-containing acids or anhydrides derived therefrom or mixtures of any, or all of the above or sulfur-containing similar acids containing aliphatic sulfur in the backbone of the acid.

The general scheme of the reaction may be described as follows:

Preformed Dispersant + Sulfur Acid  $\longrightarrow$  Desired product

Hydrocarbyl + polyol intermediate + sulfur desired  
anhydride product (dispersant) acid product  
or acid 2) (3)

(1)

A.

B.

5

Alternatively (3), the sulfur acid, may be reacted directly with (1) the hydrocarbyl anhydride or acid and the reaction product thereof is thereafter reacted with (2) the polyol. It is to be understood that (1), (2) and (3) may be simultaneously reacted if so desired.

Generally speaking, the polymeric ester is derived from an alkenyl succinic compound, i.e., an alkenyl succinic anhydride or acid. The alkenyl group can be polypropylene, polybutylene, polypentyl, oligomeric hexenyl, oligomeric oleyl, oligomeric decenes or mixtures of these or similar hydrocarbylene groups. Preferred is isobutylene succinic anhydride having a molecular weight in the range of about 300 to 3,000, how-

10

15

20

### EXAMPLE 1

#### Polymeric Ester-Thiodipropionic Acid Reaction Product

A mixture of 400 g polymeric ester in diluent oil, 100 g toluene and 9 g thiodipropionic acid were charged to a 1 liter stirred reactor equipped with heater, agitator, Dean-Stark tube with condenser and an inert nitrogen atmosphere. The reactants were heated to 170°-175° C. for about six hours until water evolution during azeotropic distillation ceased. Approximately 3 ml water was collected. The solvent was removed by vacuum stripping at about 75° C. The product was a viscous fluid containing approximately 0.4% sulfur.

The product of Example 1 was blended into a 200 second solvent paraffinic neutral lubricating oil and evaluated by catalytic oxidation test at 325° F. for forty hours with the results shown in Table I. The non-sulfur containing ester used as a reactant in Example 1 was likewise blended into the identical oil and evaluated side-by-side in the same test.

TABLE 1

| Item                                                             | Catalytic Oxidation Test                |                               |                                                     |                                                 |                           |
|------------------------------------------------------------------|-----------------------------------------|-------------------------------|-----------------------------------------------------|-------------------------------------------------|---------------------------|
|                                                                  | Additive<br>Conc.<br>In 200"<br>SPN Oil | Viscosity<br>Sludge<br>Rating | % Increase<br>In Viscosity<br>Measured<br>at 40° C. | % Increase<br>In Lead<br>Measured<br>at 100° C. | % Increase<br>Loss,<br>mg |
| 1. Example 1 - Polymeric ester treated with thiodipropionic acid | 1.0                                     | Light                         | 51                                                  | -13                                             | 0.9                       |
| 2. Polymeric ester used as reagent for Example 1                 | 1.0                                     | Heavy                         | 99                                                  | 33                                              | 2.1                       |

ever, the alkenyl moiety may contain from 20 to about 36 carbon atoms or as many as 200 carbon atoms. Molecular weight ranges of 500-1,500 are most preferred. The resulting polymeric ester after reaction with a polyol source must contain at least one free hydroxyl group, but can optionally contain additional hydroxyl and/or amine groups. Such polymers are readily available through normal commercial channels or can be prepared by known methods. The sulfur-generating species are all well known articles of commerce or can be prepared by any methods known to the art, preferred is dithiopropionic acid. The molar ratio of ester to sulfur species may vary from 1:1 to 1:0.001 with 1:0.5 to 1:0.01 being preferred. The reaction can take place at temperatures varying from about 90° to about 200° C. for about 3 to 12 hours or more generally under autogenous pressure. A solvent may be used if so desired. Any of the known hydrocarbon solvents, such as toluene, benzene, hexane and the xylenes are suitable. Diluent oil can also be used as a solvent.

The following examples and comparative data serve to illustrate the novel compositions of matter of the present invention and the marked improvement in detergent/dispersant and antioxidant corrosion properties of the hydrocarbon material containing same. It is to be understood however, that it is not intended that the invention be limited to the particular compositions containing same. Various modifications and compositions can be employed as would be readily apparent to those skilled in the art.

Samples of 200" solvent paraffinic neutral mineral lubricating oil were placed in an oven at 325° F. Present in the samples were the following metals, either known to catalyze organic oxidation or commonly used materials of construction:

- 15.6 sq. in. of sand-blasted iron wire
- 0.78 sq. in. of polished copper wire
- 0.87 sq. in. of polished aluminum wire
- 0.167 sq. in. of polished lead surface.

Dry air was passed through the sample at a rate of about 5 liters per hour for 40 hours.

As can be seen from the above data, the sulfur-containing product of Example 1 controls the increase in viscosity of the test oil at both temperatures, the lead loss due to corrosivity, and the sludge formation (a measure of dispersancy-detergency) better than equal concentrations of the identical non-sulfur containing product.

The corrosivity of the products in accordance with the present invention were evaluated as shown in Table 2.

TABLE 2

| Item                                                             | Evaluation of Corrosivity - ASTM D130-6              |                             |                    |
|------------------------------------------------------------------|------------------------------------------------------|-----------------------------|--------------------|
|                                                                  | Additive<br>Concen-<br>tration<br>In 200"<br>SPN Oil | D130-6(6 Hrs. @<br>100° C.) | Corrosivity Rating |
|                                                                  | ASTM                                                 | ASTM D130                   |                    |
| 1. Example 1 - Polymeric ester treated with thiodipropionic acid | 1.0                                                  | 1A                          | 1A                 |
| 2. Polymeric ester used as reagent for                           | 1.0                                                  | 1A                          | 1B                 |

TABLE 2-continued

| Evaluation of Corrosivity - ASTM D130-6 |                                   |                             |                    |
|-----------------------------------------|-----------------------------------|-----------------------------|--------------------|
| Item                                    | Additive Concentration<br>In 200" | D130-6(6 Hrs. @<br>100° C.) | Corrosivity Rating |
| Example 1                               | SPN Oil                           | ASTM                        | ASTM D130          |

The additive products described herein are effective in amounts ranging from 0.001 to about 10 wt. % and preferably from about 0.01 to about 5 wt. %. It is also understood that other additives for their known purposes, may be incorporated into the formulations of the present invention in amounts up to about 20 wt. % of the total composition. Included, for example, are friction-modifying, metal passivating, antiwear, bearing corrosion inhibitives, thermal stability additives and the like, metallic phenates and/or sulfonates, metallic or ashless phosphorodithioates, sulfurized olefins, polymeric pour depressants and other commonly used additives.

As can be seen from the above data, the products of the invention are excellent with respect to control of copper corrosivity despite its sulfur content as well as having excellent oxidative and thermal stabilizing characteristics.

What is claimed is:

1. A composition comprising a liquid hydrocarbyl or hydrocarbyloxy fuel and a minor dispersant/detergent and/or antioxidant amount of an additive consisting of a polymeric, oligomeric or hydrocarbyl ester containing integral sulfur-ester moieties prepared by reacting (1) a polycarboxylate ester made by the reaction of a C<sub>20</sub> to about a C<sub>200</sub> alkenyl succinic anhydride or acid and a polyol having from about 6 to about 30 carbon atoms and from about 3 to about 6 hydroxyl groups said ester containing at least one free hydroxyl group and having at least 30 carbon atoms and (2) a sulfur-containing acid or acid generating species selected from the group consisting of thiadipropionic acid, dithiopropionic acid, thiobutanoic acid, anhydrides thereof or mixtures thereof in an ester to sulfur species molar ratio of from about 1:1 to about 1:0.001 at temperatures of from about 80° to about 200° C.

2. The composition of claim 1 wherein the sulfur-containing species is thiadipropionic acid.

3. The composition of claim 1 wherein said ester is derived from the group comprising polypropylsuccinic or polyisobutyl succinic anhydrides or acids, oligomeric succinic anhydrides or acids.

4. The composition of claim 3 wherein the oligomeric succinic acid or anhydride is selected from the group consisting of hexenyl, octenyl or decenyl succinic anhydrides or acids thereof.

5. The composition of claim 1 wherein the polyol is selected from the group consisting of trimethylol propane, dipentaerythritol, tripentaerythritol tris(hydroxymethyl)aminomethane or mixtures thereof.

6. The composition of claim 1 wherein said polycarboxylate ester is derived from a polyisobutyl succinic anhydride or acid and pentaerythritol.

7. The composition of claim 1 wherein said additive is present in an amount from 0.01 to about 10% by weight of the total composition.

8. A composition comprising a major amount of a liquid hydrocarbyl or hydrocarbyloxy fuel and a minor dispersant/detergent and/or antioxidant amount of an additive product containing a polymeric, oligomeric or hydrocarbyl ester prepared by co-reacting (1) a polycarboxylate ester made by reaction of a C<sub>20</sub>-C<sub>200</sub> polyalkenylhydrocarbyl anhydride or acid thereof, oligomeric alkenylhydrocarbyl anhydrides or acids thereof, oligomeric, dimer or trimer acids or anhydrides thereof, containing at least one free hydroxyl group and (2) a sulfur containing acid species selected from sulfur-containing acids, anhydrides or mixtures thereof selected from the group consisting of thiadipropionic acid, dithiopropionic acid, thiobutanoic acid and anhydrides thereof and thereafter reacting the product of (1) and (2) with (3) a polyol having from 6 to about 30 carbon atoms and from about 3 to 6 hydroxyl groups.

9. The composition of claim 8 wherein (1), (2) and (3) are simultaneously reacted together.

10. The composition of claim 8 wherein said ester is derived from the group comprising polypropylsuccinic or polyisobutyl succinic anhydrides or acids, oligomeric succinic anhydrides or acids, oligomeric or polymeric dimer or trimer acids or anhydrides.

11. The composition of claim 8 wherein the polyol is selected from the group consisting of trimethylol propane, dipentaerythritol, tripentaerythritol (tris(hydroxymethyl)aminomethane or mixtures thereof).

12. The composition of claim 8 wherein said alkenylhydrocarbyl compound is derived from the group comprising polypropylsuccinic or polyisobutyl succinic anhydrides or acids.

13. The composition of claim 12 wherein the oligomeric succinic acid or anhydride is selected from the group consisting of hexenyl, octenyl or decenyl succinic anhydrides or acids thereof.

14. The composition of claim 8 wherein said alkenylhydrocarbyls compound are derived from a polymeric, oligomeric or hydrocarbyl ester containing integral sulfur-ester moieties prepared by reacting a polymeric, oligomeric or hydrocarbyl ester having at least 30 carbon atoms and containing at least one free hydroxyl group and said sulfur-containing acid or acid generating species in an ester to sulfur species molar ratio of from about 1:1 to about 1:0.001 at temperatures of from about 80° to about 200° C.

15. The composition of claim 8 wherein said reactant containing at least one free hydroxyl group is selected from the group consisting of trimethylol propane, pentaerythritol, dipentaerythritol, tripentaerythritol tris(hydroxymethyl)aminomethane or mixtures thereof.

16. The composition of claim 15 wherein said polycarboxylate ester is derived from a polyisobutyl succinic anhydride or acid and pentaerythritol.

\* \* \* \* \*